

Dec. 23, 1969

G. CERUTTI

3,485,984

METHOD FOR HEATING A THERMOPLASTIC THREAD

Filed Feb. 20, 1968



INVENTOR.  
GIACOMO CERUTTI.  
BY

Mason, Porter, Diller, Brown  
ATTORNEYS

1

3,485,984

## METHOD FOR HEATING A THERMOPLASTIC THREAD

Giacomo Cerutti, Gozzano, Novara, Italy, assignor to Bemberg S.p.A., Milan, Italy, a corporation of Italy

Filed Feb. 20, 1968, Ser. No. 709,165

Claims priority, application Italy, Mar. 4, 1967,  
13,368/67

Int. Cl. H05b 5/00, 9/00

U.S. CL. 219—10.41

7 Claims

### ABSTRACT OF THE DISCLOSURE

Method for the reduction of the residual shrinkage of thermoplastic threads wherein the thread wound on a supporting member is subjected to an RF electric field.

This invention relates to a method for heating a thermoplastic thread and, more particularly, to a method for reducing the residual shrinking of a thermoplastic thread wound on a supporting tube in the form of a spool. The invention is particularly applicable to thermoplastic threads made of linear polyamides, such as those obtained by the condensation of aminocarboxylic or bicarboxylic acids with diamines, or those made with linear polyesters such as polyethylene terephthalate. It is known that threads made with linear polymers as mentioned above, such as obtained with the melt spinning method and subsequent drawing in the solid state, have usually an intrinsic shrinkability, or residual shrinking, when they are treated with water which has been heated to a temperature in the neighbourhood of 100° C. This is tantamount to saying that a given thread sample, immersed in hot water in a relaxed condition, will exhibit a shrinking in the longitudinal direction.

Such a shrinkage is a considerable disadvantage, in that it reduces the tensile strength of the thread and gives rise to an uneven molecular orientation. In addition, the fabrics prepared with the highly shrinkable threads aforementioned, when they are subjected to heat treatments with steam, or to washing treatments at high temperatures, undergo an undesirable reduction of their dimensions. To do away with this drawback, several methods have been suggested for reducing the thread shrinkage beforehand, that is, prior to employing it in fabrics. Two of the generally adopted methods to this purpose consist of subjecting the thermoplastic thread, immediately upon drawing, to a heat treatment by causing it to slide over a pin or a similar heating member, while the length of the thread is kept constant. The thread treated in this manner is then collected on the usual spool, from which it can be drawn and processed in the usual way. Even though this method is a fairly satisfactory solution from an economical standpoint, in that it permits that the conventional machinery may be used with appropriate modifications, it is nonetheless only partly satisfactory, inasmuch as the residual shrinkage is still rather high.

Thus, for example a Nylon 6 thread, after the treatment recalled above, still retains a residual shrinkage of about 7%, whereas a still lower value would be desirable.

On the other hand, a lower residual shrinkage could be obtained by subjecting the thermoplastic thread to particular treatments, such as a heat treatment with water or a treatment with steam under pressure in an autoclave. In order to carry out these treatments, however, it is necessary to transfer the thread from the spool as obtained with the draft process to another package which is adapted to said treatments. It is obvious, then, that a method of this kind, even capable of giving satisfactory results, is rather cumbersome and expensive.

2

It has now been found that a satisfactory reduction of the residual shrinkage of a thermoplastic thread can be obtained, especially a thread made with linear polyamides or linear polyesters, wound on a tubular supporting member in the form of a spool, if the supporting member for the wound thread is used as the dielectric between two electrodes energized by an RF voltage, having an RMS value ranging between 1,000 and 2,000 volts and a frequency comprised between 10 and 200 megacycles and a service capacity comprised between 2 and 6 kilowatts for a time from 1 to 10 minutes.

The thread is thus subjected to the influence of an RF field and becomes gradually heated, so that it undergoes a heat treatment while its length remains substantially constant. The spools of thread to be subjected to the treatment can be the same as obtained through the performance of the drawing process, and this fact is a considerable advantage of the inventive method. After the treatment, the thermoplastic thread can be used as such by taking it out of the spool. Its residual shrinkage will be in the range from 1% to 4% according to the intensity of the treatment and the nature of the polymer. It should be noticed that, with the inventive method, the heat treatment of the thread spool takes place in a uniform manner throughout the entire mass of the thread, that which also ensures a regular trend of the shrinkage throughout the entire length of the thread. A heat treatment which, instead, should be carried out with an external heat source, such as subjecting the thread spool to the action of infrared radiations, would give rise to a temperature differential within the thread mass, in that the outermost layer of the spool would be heated more rapidly than the inner layers, the result being an unevenness of the residual shrinkage throughout the entire thread length. In addition, on account of the poor thermal conductivity of polyamides and polyesters, this indirect heating method would be rather slow.

As a generator of the RF field and conventional device can be used, provided, of course, that it has the specifications indicated above. The field electrodes should be so shaped as to match the particular form of the thread spool to be treated.

Thus, if the thread spool has been formed on a metal supporting tube, as is the case when the as drawn thread is collected with the dressing ring method, then the supporting tube itself can be used as either field electrode, whereas the second electrode will be a tube having a diameter slightly greater than the overall diameter of the thread spool. The metal tube which supports the thread spool, as it should be used as an electrode, will be preferably made of aluminium. It is possible, however, to use tubes made of other metallic materials, for example, steel. It should be born in mind, however, that materials such as steel, when they are used as electrodes and are energized by an RF voltage, tend to become rapidly heated, a fact which could be conducive to drawbacks of various nature.

At any rate, the second electrode will be preferably made of copper.

If, conversely, the thread spool has been formed on a non-metallic cylindrical supporting member, for example, paper or a synthetic resin, as is the case when the collection of the as drawn thread is carried out on a rotary drum into which the supporting member has been slipped, then two confrontingly mounted electrodes will be required, placed in contact with the two sides of the thread spool and preferably made of copper.

Be it understood, in any case, that thread spools having a shape other than that described herein can be subjected to the inventive treatment: consequently, field electrodes having a configuration suitable for such forms

of packing will be used without departing from the scope of this invention.

The invention will be now explained with reference to the accompanying drawings which are not to be construed as limitations.

FIGURE 1 is illustrative of an embodiment of the inventive method, in which the thread to be subjected to the action of the RF field is wound on a metal tube.

FIGURE 2 shows another embodiment, in which the thread to be subjected to the RF field is wound on a non-metallic cylindrical supporting member, and

FIGURE 3 is a cross-sectional view of the thread spool and the RF field electrodes shown in FIG. 2.

Having now reference to FIG. 1, the numeral 1 indicates either field electrode, having a cylindrical configuration. The thread spool 2 is placed in the interior of said electrode. The metal tube 3, on which the thread is wound, acts as the second field electrode. The electrodes 1 and 3 are stuck into the supporting plate 4, in the interior of which they are connected to the coaxial leads 5 and 6 through which the RF voltage, as produced by a generator, not shown in the drawing, is fed.

Having now reference to FIGS. 2 and 3, the electrodes 1 and 2 are so shaped as to exhibit annular projections 3 and 4. The thread spool 5, having a cylindrical supporting member 6 made of a non-metallic material, is positioned between the electrodes 1 and 2 so that its sides directly contact the annular projections 3 and 4 of the electrodes. In addition, to the electrodes 1 is affixed a cylindrical block 7, of a non-metallic material, intended to support the spool 5. The electrodes 1 and 2 have, on their bottom portion, two coaxial plugs 10 and 11 which permit to insert into, and withdraw from the coaxial sockets 8 and 9 formed in the supporting plate 12, the electrodes and spool assembly.

The coaxial plugs 8 and 9 are connected, in the interior of the bedplate 12 (this detail is not shown in the drawing), to the coaxial leads 13 and 14, through which the RF voltage, supplied by a generator not shown in FIG. 2, is fed in.

This invention is not limited, however, to the embodiments shown therein. Continuous treatment processes could be envisaged without departing from the scope of the invention. Thus, for example, the thread spools could be arranged in a horizontal row on a conveyor belt or another like member which, being moved in a continuous run, causes the thread spools sequentially to be passed between two confronting plate electrodes, energized by a RF voltage having the specifications provided for by the present invention, the spatial velocity of the spool being calculated so that each individual portion of the spool is subjected to the heat treatment for a time whose duration is roughly the one which is required in the treatment at standstill for producing an acceptable reduction of the residual shrinkage.

The invention will be now illustrated by the following practical examples which have no limiting value whatsoever.

#### EXAMPLE 1

A 15-filament caprolactam thread was drawn and immediately after wound, according to the ring dressing method, on a support formed by an aluminium tube having a length of 370 mms. and an outside diameter of 50 mms. The denier of the drawn thread was 60 and the residual shrinkage of the thread was about 14%, as measured on a skin of 100 meters of thread subjected to boiling in water for 30 minutes and then dried.

The net weight of thread wound on the spool was about 1.6 kgs. The spool was wound with a gradual reduction of the stroke of the ring rail, so that, from an initial length of stroke of 330 mms., a final length of stroke of 185 mms. was obtained. The maximum diameter of the spool was 115 mms. The thread spool so prepared was subjected to an RF field, by using an apparatus similar to that shown in FIG. 1 hereof. The alu-

minium tube forming the support of the spool was used as a field electrode by connecting it to a coaxial lead, whereas the second electrode was a copper cylinder having an inside diameter of 117 mms. and a length of 405 mms., in the interior of which the thread spool was positioned.

The copper electrode was connected to a second coaxial lead which, along with the first one, provided the energization of the electrodes. Both the aluminium tube and the copper cylinder were placed on an appropriate pedestal. The whole assembly had to be shielded in order to avoid interferences towards the outside of the field so produced. A driving cab, supplying a service capacity of 6 kilowatts, supplies the electrodes with an RMS voltage of 2,000 volts at a frequency of 75 megacycles. After 2 minutes the treatment was discontinued and the thread spool withdrawn.

The residual shrinkage of the thread was measured by taking samples from the several layers of the wound spool: the result was that the residual shrinkage varied from 2.5% to 3.5%.

#### EXAMPLE 2

A caprolactam thread spool having the same specifications as that of Example 1 was subjected to a heat treatment by using the same implementation adopted for the previous example, the only difference being that a power of 4 kilowatts, an RMS voltage of 1,300 volts and a frequency of 110 megacycles were used. The duration of the treatment was again 2 minutes.

Thread samples, taken from several layers of the wound spool, gave a residual shrinkage which varied within the same range as in Example 1, that is, from 2.5% to 3.5%.

#### EXAMPLE 3

A polycaprolactam thread spool, having the same characteristics as in Example 1, was subjected to heat treatment by using the same implementation as used in Example 1, the only difference being that the driving cab had a power of 4 kilowatts and fed the electrodes with an RMS voltage of 2,000 volts at a frequency of 10 megacycles. The implementation had not to be shielded. After 10 minutes the treatment was discontinued and the thread spool withdrawn. The residual shrinkage of the thread was measured by taking samples from the several layers of the wound spool and the residual shrinkage was found to vary between 3.5% and 4.5%.

#### EXAMPLE 4

A polyhexamethylene adipamide thread composed by 10 filaments was drawn and collected on a non-metallic cylindrical supporting member slipped into a rotary drum.

The cylindrical supporting member had a diameter of 100 mms. and a height of 150 mms.

The thread, the final denier of which was 50, was wound on the supporting member in the form of a spool having a width of the wound thread of 100 mms. and a thickness of 110 mms. The net weight of the thread was 1.8 kgs.

The thread spool so prepared was subjected to a heat treatment by means of the implementation shown in FIG. 2.

The gap between the two field electrodes was thus 100 mms., equal to the width of the wound spool.

The electrodes were energized by an RMS voltage of 1,500 volts at a frequency of 110 megacycles and a power of 4 kilowatts.

The treatment lasted 3 minutes.

Thread samples, taken from several layers of the wound spool, gave a residual shrinkage which varied from 1% to 2%, as compared with the residual shrinkage of 11% of the untreated thread.

#### EXAMPLE 5

A 18-filament polyethylene terephthalate thread was drawn and collected on a non-metallic cylindrical support,

inserted into a rotary drum having the same size as that of Example 4. Also the size of the thread spool, the final denier of which was 48, was the same as in Example 4.

The spool was positioned in the same implementation used for treating the polyhexamethylene adipamide and a heat treatment was carried out by energizing the electrodes with an RMS voltage of 1,200 volts at a frequency of 150 megacycles and a power of 6 kilowatts. The treatment lasted 150 seconds.

Thread samples, taken from several layers of the wound spool, gave a residual shrinkage of from 2% to 3%, as compared with an 8% shrinkage of the untreated thread.

While in the disclosure of this invention reference has been made to thermoplastic threads, and more particularly to those made of linear polyamides and polyesters, the invention is not to be regarded as being limited to said threads only. In point of fact it will be possible, as a rule, to apply the inventive method also to other thermoplastic threads for which a direct heat treatment on the spool is desirable for any reasons, such as to polyolephine, poly- 20 urethane and polyvinyl threads.

What is claimed is:

1. A method of reducing residual shrinkage of thermoplastic thread wound on a metal spool comprising the steps of positioning the wound thread as a dielectric between two electrodes, one of the electrodes being the metal spool upon which the thread is wound, and heating the thread by energizing the electrodes with an RF voltage. 25

2. The method of claim 1 including providing a metal tube as the other electrode.

3. The method of claim 2 including completely surrounding the wound thread with the metal tube.

4. The method of claim 1 wherein the RF voltage has an RMS value of from 1,000 to 2,000 volts, a frequency between 10 and 200 megacycles, and a service capacity between 2 and 6 kilowatts, for a time of from 1 to 10 minutes.

5. The method of claim 1 wherein the metal spool is made of aluminum.

6. The method of claim 1 characterized in that the thermoplastic thread is made of a linear polyamide.

7. The method of claim 1 characterized in that the thermoplastic thread is made of linear polyester.

10

15

20

25

30

2,421,334 5/1947 Kline et al. ----- 219—10.81  
2,433,842 1/1948 Griffin ----- 219—10.41  
2,479,351 8/1949 Hagopian ----- 219—10.81 X  
2,635,352 4/1953 Phillips ----- 219—10.41 X  
2,866,063 12/1958 Rudd ----- 219—10.81 X  
2,364,294 1/1968 Garibian et al. --- 219—10.61 X

JOSEPH V. TRUHE, Primary Examiner

L. H. BENDER, Assistant Examiner

#### U.S. Cl. X.R.

34—1; 219—10.61, 10.81

#### References Cited

#### UNITED STATES PATENTS